

March 4, 1958

K. BAUM

2,825,679

## BRIQUETTING OF COKE BY DIRECT HEATING

Filed June 16, 1953

3 Sheets-Sheet 1



**INVENTOR.**

KURT BAUM

BY  
Caryell, Newburgh, Freed & Graves  
HIS ATTORNEYS.

March 4, 1958

K. BAUM

2,825,679

BRIQUETTING OF COKE BY DIRECT HEATING

Filed June 16, 1953

3 Sheets-Sheet 2



INVENTOR  
KURT BAUM

BY  
Campbell, Brumbaugh, Freer & Graves  
ATTORNEY

March 4, 1958

K. BAUM

2,825,679

## BRIQUETTING OF COKE BY DIRECT HEATING

Filed June 16, 1953

3 Sheets-Sheet 3



INVENTOR.  
KURT BAUM

BY  
Cayleb Brewbaker, Esq. & Geaves  
HIS ATTORNEYS.

1  
2,825,679

## BRIQUETTING OF COKE BY DIRECT HEATING

Kurt Baum, Sevres, France

Application June 16, 1953, Serial No. 362,007

Claims priority, application France March 30, 1948

8 Claims. (Cl. 202—26)

The present invention relates to methods and apparatus for the production of coke and especially metallurgical coke.

This is a continuation-in-part of my application Serial No. 81,195, filed March 12, 1949, now abandoned, and of my application Serial No. 95,276, filed May 25, 1949, now abandoned.

In the usual coking plants, in which the coal to be coked is heated indirectly, i. e. by heat conduction through the partitions of the coking chambers, relatively low daily outputs are obtained in each chamber, because heating is necessarily slow (rate of temperature rise ranging from 1° to 2° C. per minute). Furthermore, even if this rate of temperature rise during heating of the coal to be coked could be improved, the coke obtained would be too small and too brittle.

It is also known, in order to obtain fully degasified cokes, to submit to full coking treatment agglomerates at least partly composed of coal having already undergone a first partial carbonization. However, this method has for its only purpose to permit the use of coals other than coking coal for the production of coke. It does not remedy in any way the slowness of the heating action during coking, which slowness limits the daily output of the coking chambers. Furthermore, this process calls for relatively large quantities of binder, for example tar or pitch, in order to produce agglomerates suitable for high temperature full coking.

Finally, it is also known to produce semi-cokes by heating agglomerates of coal through direct contact with a heating gas, with a relatively quick rise of the temperature. However, this process cannot be used for obtaining fully degasified coke through coking at high temperature because coke obtained in this way is too fine and too brittle.

One object of my invention is to provide a coking plant capable of producing, per unit of time, a higher amount of coke than it was possible with prior methods and apparatus.

Another object is to obtain coke, and in particular, high quality coke, from fuels which up to now were not considered suitable for this purpose.

In accordance with my invention, I obtain cokes of high mechanical strength, suitable for metallurgical and other uses at high production rates by bringing unheated agglomerates or briquettes (containing less than 20% volatile materials and made from semi-cokes produced from natural or artificial coals) into direct contact with highly heated gas to cause an average temperature rise in the briquettes or agglomerates of 5° C. to 15° C. per minute.

It is particularly advantageous to make the agglomerates or briquettes chiefly of a semi-coke obtained from coal of an indefinite geological age (lignite, brown coals, sub-bituminous coal, high volatile bituminous coal, B and C rank), or even charcoal from wood or peat, which semi-coke is mixed with coking or swelling coal and with a binder such as tar or pitch and molded to form the agglomerates or briquettes.

5 The rate of average temperature rise of the agglomerates to be coked under the aforesaid conditions depends further upon the dimensions of these agglomerates. For instance, in the case of briquettes of a weight of 1,000 grams per briquette, it ranges from 5 to 7.5° C. per minute. In the case of briquettes of a weight of 250 gr. per briquette, it ranges from 10 to 15° C. per minute.

10 Experience has proved that simultaneous use of a percentage of volatile matter of the briquettes corresponding to the values above mentioned and of such a quick rise of the temperature of the agglomerates, from an unheated or cold state, makes it possible to obtain cokes of high mechanical strength. The quick rise of temperature causes melting and coking of the fusible matters contained in the agglomerates before these can decompose and be driven off as volatile vapors. The same phenomenon is the reason why I can make use of agglomerates containing but relatively small quantities of binder to produce cokes of high mechanical strength.

15 The coke obtained according to my invention has remarkable properties, and in particular its hardness, mechanical density and the uniformity of dimension of its elements, which corresponds to the dimensions of the agglomerates prior to undergoing the coking treatment. 20 As a matter of fact, this coke, tested by tumbling the coke in a drum, resists breakage in the proportion of 85% to 90%. It can be utilized for all kinds of purposes, for example for blast furnaces, cupola furnaces, for the production of watergas, etc. Concerning blast furnaces in 25 particular, very satisfactory results were obtained with coke made according to my invention from agglomerates, the semi-coke of which had been obtained for example from lignite.

30 In foundries, the coke produced according to my invention gave better results than those obtained up to now with the best special foundry coke. As a matter of fact, the use of coke made according to my invention, without giving rise to an increase of fuel consumption, made it possible to obtain a cast iron having physical qualities 35 superior to those of cast iron obtained with the best known special foundry coke. This result is probably due to the possibility of using, for producing coke according to my invention, non-coking coals of relatively recent geological age, producing residues of a high capacity of reaction.

40 45 When agglomerates (briquettes or ovoids) of natural and/or artificial coal are coked by causing heating gas to flow directly through the mass of agglomerates to be coked, this gas leaves as a typical result of my invention the coke oven with a temperature of 750 to 850° C., i. e., 50 still rather high so that it can be used in the distillation of coal fines or coal powder for the production of semi-coke or for other purposes.

55 For a better understanding of the present invention, reference may be had to the accompanying drawings in which:

Fig. 1 is a diagrammatic illustration of a typical installation for producing coke in accordance with my invention; and

Fig. 2 is a diagrammatic illustration of a modified installation for practicing the invention.

Fig. 3 similarly shows still another installation according to my invention.

60 65 In accordance with the present invention, coke of high quality can be produced from many types of normally non-coking coals by suitably treating such coals in a finely divided form. The finely divided coal is subjected to a preliminary distillation in direct contact with heated gas to bring the coal to a temperature of 300° C. to 550° C. and thereby drive off the volatiles and produce a semi-coke having between 9 and 12% volatiles. It is particularly important with lignites and other similar coals

which have poor coking properties to reduce the volatile content at least down to 12%, as otherwise the coke produced therefrom is brittle and of low mechanical strength.

The semi-coke produced as described above is cooled and is formed into agglomerates or briquettes by mixing it with a small amount of binder such as pitch and a small amount of swelling type coal. By way of example such agglomerates may be composed of about 80% semi-coke, 15% of finely ground swelling or coking coal and about 5% of pitch.

The briquettes or agglomerates are then introduced without preliminary heating, directly into a coking retort where highly heated gases (1,000° C. to 1,250° C.) are brought into contact with the briquettes or agglomerates. The flow of gases between the briquettes in the retort preferably is crosswise to the direction of movement of the briquettes so that they will be heated strongly and uniformly and will increase in temperature at a rate of 5° C. to 15° C. per minute. The rate of temperature rise of the briquettes to be coked depends upon the dimensions of the briquettes, which preferably have a weigh between about 1000 and 250 grams per briquette.

Due to the rapid heating of the briquettes the time required for producing the fully coked material is greatly reduced and, moreover, a higher quality product results. The rapid increase in temperature apparently converts the binder and other volatiles into a coke-like material which seals the briquettes and prevents loss of the binder and other volatiles with the result that the carbon particles of the briquettes are bonded strongly together to produce coke of high mechanical strength and with a minimum of cracking or shattering.

The drawings illustrate typical installations with which the method can be practiced.

The distillation apparatus  $T_1$  diagrammatically shown by Fig. 1 is typical of those which may be used for producing the semi-coke. Distillation takes place in the apparatus  $T_1$  by direct contact of coal fines or coal powder with the heating gas. This apparatus includes one or several chambers, for example two chambers  $102'$  and  $102''$  connected together in series, through which passes the stream of heating gas into which are injected at  $103$  the coal fines or powders to be distilled. These coal fines or powders are supplied from a tank  $VA$ ; they are dried in a dryer  $XA$  by means of a stream of hot gas from which they are separated in cyclone  $118$ , after which they are conveyed through a pipe  $119$  to the coal fine inlet  $103$  of the element  $102'$  of distillation apparatus  $T_1$ . These fines or powders are carried along by the heating gas stream coming from coke oven  $A$  in which they are in suspension and they pass through the two distillation chambers  $102'$  and  $102''$ . Simultaneously with this, coal distillation takes place under the action of the sensible heat of the heating gas. A portion of the semi-coke thus formed deposits at the bottom of chamber  $102''$  of distillation apparatus  $T_1$ , whereas the remainder, carried along by the heating gas to the outside of this chamber  $102''$ , is separated from the gas within a cyclone or the like  $104$ .

This semi-coke is then cooled, preferably by introducing it into a cooling gaseous stream, as shown by Fig. 1. Said semi-coke coming both from cyclone  $104$  and from the bottom of distillation chamber  $102''$  is fed, through pipe  $105$ , into a gaseous cooling stream driven by a blower  $105'$ , this stream passing, after it has been mixed with the semi-coke, through a heat interchanger  $L$  where the semi-coke is cooled and the gaseous stream from blower  $105'$  gets heated. Upon leaving this heat interchanger  $L$ , the cooled semi-coke is separated from the carrier gas in a cyclone or the like  $115$ , whereas the gas, heated up in  $L$  by the heat of the semi-coke, is advantageously utilized for drying in dryer  $XA$  the coal fines or powder from tank  $VA$  to be subjected later on to low temperature distillation.

The semi-coke thus cooled is utilized for the production of agglomerates or of briquettes in a press  $116$  (Fig. 1). These agglomerates preferably consist of a mixture of the semi-cokes in question with finely ground swelling or coking coal and pitch, the total content of volatile matter of this mixture being lower than 20%. These agglomerates are then carried by a conveying system, for example an elevator  $117$ , to the charging hopper of coke oven  $A$ .

Said coke oven  $A$  includes an outer shell  $3$ , a vertical shaft  $1$  inside said shell and two horizontal partitions which divide the space between said shaft  $1$  and said shell  $3$  into two chambers for the passage of gases, to wit, an upper chamber and a lower chamber. The agglomerates are dropped at  $2$  into shaft  $1$  and the coke leaves it at  $7$ . Of course, in order to enable the gases to pass through the material travelling downwardly through shaft  $1$ , the wall of said shaft, in the portions thereof located in the above mentioned chambers, is provided with apertures, for instance so as to be of grate-like structure, as conventionally shown by the small rectangles visible in Fig. 1 and which are designated by reference numerals  $5$  and  $6$  for the upper chamber.

The coking zone of oven  $A$  is constituted by this upper chamber. The heating gas stream (at a temperature between about 1000° C. and 1250° C.) enters this chamber on the right hand side thereof (for instance from a regenerator such as  $O$  as it will be hereinafter described). This gas stream, after passing through the mass of agglomerates which are travelling downwardly through the portion of shaft  $1$  located in said upper chamber, flows out (according to the path shown by the dotted lines) toward the left to pass into conduit  $103$ .

As already stated, according to my invention, the flow rate of the heating gas stream passing through the coking zone of oven  $A$  and that of the stream of briquettes or agglomerates passing in shaft  $1$  through said zone are adjusted so that said briquettes, which are introduced at  $2$  without preheating, are heated, during their passage through said coking zone (upper chamber of oven  $A$ ), at a rate of 5° C. to 15° C. per minute, whereas the temperature of the heating gas stream drops from 1000-1250° C. on the right hand side of the upper chamber of oven  $A$  down to 750-850° C. in conduit  $103$  (of course it should be well understood that these values are average values).

Owing to this quick rise of the temperature of the briquettes or other agglomerates in the coking zone of coke oven  $A$ , the coke output per square meter of the coking chamber area is equal to several times the best yields yet obtained up to now. With the best vertical coking plants known up to now, in which the agglomerates pass continually through a coking chamber heated from the outside, and cooling chambers for direct gas contact, an output of 20-22 kgs. of agglomerates per square meter of coking chamber area and per hour, was the maximum that could be obtained, whereas, in an oven as shown by the drawing and working according to my invention, yields of 150 to 200 kgs. of agglomerates per square meter of coking chamber area and per hour are obtained.

With my invention, I therefore obtain, for the same oven measurements, a daily output of wholly gas-free coke from seven to nine times greater than the yield of the best plants known up to now.

Another advantage lies in the fact that a plant made according to my invention, using no silica bricks, can be stopped and restarted at any time. Restarting can take place immediately if the heating of the regenerators has been maintained. If not, restarting necessitates a delay of 10 to 12 days necessary for re-heating the said generators, which is an extremely short time as compared with those necessitated for restarting plants known at the present time.

As a rule, it is advantageous as in the example above

described, to pre-dry the coal powders or coal fines before introducing them into the low temperature distillation plant. This drying, which may be carried out in any appropriate manner, is preferably performed in devices through which the coal fines or coal powder are carried along by a carrier gas.

In the plant shown by Fig. 1, the carrier gas circulating through dryer XA flows through the following closed circuit: Blower 105', heat interchanger L where the gas is heated by the semi-coke circulating therewith, cyclone 115, where the gas is separated from said semi-coke, then dryer XA, cyclone 118 and once more blower 105'.

Another drying device for coal fines or coal powder is shown by Fig. 2. In this case, the coal to be dried is also introduced into a gaseous stream circulating in a closed circuit and driven by blower M. The mixture of this gaseous stream and coal powder or coal fines to be dried passes through the tubes of a dryer XA', externally heated by a heating fluid which also passes through this dryer XA'. Upon leaving XA', the now dried coal fines and coal powder are separated from the gaseous carrier flow by means of a plurality of cyclone type separators 118'. This gaseous carrier is returned from separator 118' to blower M as shown by the dotted lines.

Every time coal fines or coal powder are dried in a carrier gas circulating in a closed circuit, the steam and the excess of gas formed by this drying process have to be withdrawn from the carrier gas at N (Fig. 1 and Fig. 2).

Finally, it should be noted that the heating up of the portion of the coking gas that is reintroduced into coke oven A, besides being performed by direct internal combustion, may be obtained, as shown in the plants of Figs. 1 and 2, by means of two regenerators (such as that shown at O) inserted alternately in the flow of gas to be heated up and in a flow of fluid intended to heat up the regenerators. The coking gas to be heated up passes successively through one of these regenerators O, coke oven A, the distillation apparatus, then a pitch separator P, a cooler Q, a blower R and possibly other apparatus intended to purify the gas and to recover any recoverable matters contained therein. After passing through all these apparatus, a portion of the gas, forming the surplus, is withdrawn from the circuit at S, whereas either the whole of the remainder returns to the regenerator (Fig. 2) or only a portion of this remainder returns to the regenerator and the other portion flows to the lower chamber 1a of coke oven A (Fig. 1). In this latter case, the two gaseous streams join together before re-entering the distillation apparatus T<sub>1</sub>, the gaseous stream which flows through said lower chamber 1a being heated by interchange of heat with the coke travelling through the central shaft of said chamber and which is thus cooled.

I may advantageously obtain low temperature distillation of coal fines or coal powder by injecting them into a portion of the gas coming from this distillation apparatus and circulating in a closed circuit. This gas, after leaving the distillation apparatus, and being separated from the semi-coke produced by distillation, is freed from its recoverable by-products, such as pitch or tar and finally heated by means of an external source. This source is totally or partly constituted by the sensible heat of the gas coming from the directly heated coke oven.

Thus, in the construction illustrated by Fig. 2, coal fines or coal powders from separator 113' are injected at J into a low temperature distillation apparatus T<sub>2</sub> to mix with a stream of hot gas which enters said apparatus at 106 and leaves it at 107. The coal fines or coal powders mixed with this gas stream are carried along through the pipes 111 of apparatus T<sub>2</sub>. These pipes are externally heated by gases coming from coke oven A through pipe 103. These gases enter the apparatus T<sub>2</sub> at 109 and leave it at 110 so that heating truly takes place in countercurrent fashion.

The gas stream that leaves at 107, enriched with the

low temperature distillation gas and which carries along the semi-coke formed during distillation, passes through cyclone 112, where semi-coke is separated from this gas stream. The gas, thus freed from semi-coke, flows through a cooler V acting at the same time as a pitch separator, and through a light-oil separator W, a blower B which returns a portion of this distillation gas through pipe 113 into distillation apparatus T<sub>2</sub> and sends the other portion through pipe 114 into a gas tank.

According to another feature of my invention which may be used separately, the heating of coal fines or coal powder is ensured both in countercurrent fashion and in equi-current fashion at the same time in the low temperature distillation apparatus T<sub>2</sub>. For this purpose, as shown by Fig. 2, the portion of the distillation gas re-introduced into the distillation apparatus at 106 is heated, so that the coal fines or coal powder injected at J into the distillation gas immediately undergo a rise of temperature produced by the sensible heat of this gas, thus ensuring an equi-current heating, whereas the coking gas supplies through 108, 109 the indirect countercurrent heating in the above-described manner.

In order to pre-heat the portion of the distillation gas that enters at 106 distillation apparatus T<sub>2</sub>, I preferably utilize the heat of the coke of the lower part 1a of coke oven A. For this purpose, the distillation gas collected through pipe 113 is made to flow through part 1a of said chamber in order to heat the gas by contact thereof with the coke, whereas this coke is cooled at the same time.

30 The gas is thus preheated to a temperature of about 300° C.

It should further be noted that the coking gas leaving coke oven A at K is used for the external heating of the pipes 111 of distillation apparatus T<sub>2</sub> and has, on entering this apparatus T<sub>2</sub>, a temperature of about 700°-800° C.

35 The surplus gas discharged through the pipe 114 is a power gas having a heating power ranging from 3,000 to 3,500 kilogram calories per cubic meter. This gas may be utilized as it is, or, if the distillation gas is obtained separately, both gases may be mixed to form an illuminating gas having a heating power ranging from 4,000 to 4,500 calories.

40 Fig. 3 shows an installation according to my invention chiefly characterized in that the heating gas passing through coking oven A<sub>1</sub> is made to flow transversely to the direction of travel of the stream of agglomerates now in one direction now in the opposite one.

45 In this case also, the agglomerates to be treated are first subjected to quick coking by passing through a layer of these agglomerates present in vertical coking shaft or chamber 1 heating gases which flow in through the apertures of one of the vertical walls of chamber 1 and out through the opposed wall thereof. The agglomerates to be coked enter shaft 1 at its upper end and leave it, after 50 they have been fully coked, at the lower end thereof. As above indicated, heating must be sufficiently fast to obtain very quickly, on every agglomerate, a coked crust of a relatively high mechanical resistance. The fully coked agglomerates will be constantly removed at the 55 bottom of coking chamber 1.

50 This heating gas, which flows through the coking shaft 1 of the coking oven A<sub>1</sub>, is constituted by a portion of the gases obtained by coking itself, which portion is made to flow in a closed circuit, so that it passes successively 55 through a dust separator 22, a pitch separator P, a cooler Q, a blower R, possibly a second cooler Q', a benzol separator 26, a gas reservoir 28 and a reheating device constituted, for instance, by two regenerators O, O' alternately brought into play and from which the re-heated gas 60 is reintroduced into the coking furnace.

55 In this way, I recover all the by-products contained in the coking gas and I may withdraw from reservoir 28 the excess of coking gas which is not reintroduced into the coking oven and which constitutes a gas of high calorific power to be used, for instance, as town gas.

In this form of my invention, I provide means for periodically changing the direction of the heating gases that pass through the agglomerates in coking chamber 1, whereby the gases flow through these products once for instance from left to right and then from right to left, again from left to right, and so on.

This operation is advantageous because the agglomerates to be coked should be heated in a manner as uniform as possible over the whole width of the coking chamber. This condition determines the maximum drop of temperature that can be undergone by the heating gases when passing through the mass of agglomerates to be coked and, consequently, the maximum width of coking chamber 1. When the heating gases pass through the mass of agglomerates always in the same direction and if the maximum admissible drop of temperature of the heating gases is supposed to be about 200° C. (for instance from 1000° C. to 800° C.), the width of chamber 1 should not exceed values ranging from 400 to 800 mm. If, on the contrary, the direction in which the gases flow through the coking chamber is changed periodically, for instance every ten minutes, the width of this chamber can be approximately doubled, i. e. this width could, in the example that is being considered, reach values ranging from 800 to 1200 mm. In other words, it will be possible to double the capacity of the coking chamber.

The coking chamber shown by Fig. 3 is arranged to permit periodical changing of the direction of flow of the heating gases which pass through the mass to be coked. For this purpose, it includes, on either side of chamber 1, two inlets 11 and 12 for the heating gas, which communicate respectively with regenerators O and O'. Furthermore, it includes, also on either side of chamber 1, two heating gas outlets 13 and 14, both connected to conduit 15, which convey the exhaust gases from the coking oven to dust separator 22. I further provide, in each of the heating gas inlets and outlets, control means constituted for instance by mere shutters 16, 17, 18 and 19, which enable the heating gases either to enter through 11 into the coking oven and to leave it through 14, after having passed through coking chamber 1 in a left to right direction, or to enter through 12 into the coking oven and to leave it through 13, after having passed through coking chamber 1 in a right to left direction. Operation of these shutters is advantageously coupled with that of the control means provided at 20 to send the heating gases withdrawn from reservoir 28 alternately into regenerator O and into regenerator O'. I thus produce simultaneously, for instance every ten minutes, both a change in the regenerator in service (the other one being thus given time to be re-heated) and in the direction of flow of the heating gases through the mass to be coked.

While I have, in the above description, disclosed what I deem to be practical and efficient embodiments of my invention, it should be well understood that I do not wish to be limited thereto as changes might be made in the arrangement, disposition and form of the parts without departing from the principle of the present invention as defined in the following claims.

What I claim is:

1. The method of producing metallurgical coke from briquettes consisting of semi-coke, a small percent of swelling-type coal and a binder, with not more than 20% volatile components, comprising advancing a stream of said briquettes without substantial pre-heating in one direction, directing a stream of heating gas through said stream of said briquettes to cause the gas to come into direct contact with each briquette, said heating gas being heated to a temperature between about 1,000° C. and 1250° C., to heat said briquettes at an average temperature rise between about 5° C. and 15° C. per minute to a coking temperature of about 950° C., to convert the briquettes to coke while the mean temperature of the contacting heating gas is reduced to between about 750° C. and about 850° C., and cooling said briquettes.

2. The method of producing metallurgical coke which comprises heat-treating a mass of finely divided carbonaceous material to semi-coke the same, mixing the semi-cooked material with a finely divided, swelling type coal and a binder, shaping the mixture into relatively uniformly sized agglomerates containing less than twenty percent of volatile substance, advancing said agglomerates in an initially substantially unheated state in a continuous stream flowing in one direction, directing a stream of heating gas at a temperature between about 1,000° C. and about 1,250° C., through said stream of agglomerates in direct contact with the agglomerates therein and transversely to said direction of movement of the stream of agglomerates, the rate of flow of said stream of agglomerates being such that they are heated at an average temperature rise of about 5° C. to 15° C. per minute to about 950° C. after passage of the said heating gas stream therethrough while the mean temperature of the contacting heating gas is reduced to between about 750° C. and about 850° C. and utilizing the said reduced temperature heating gas for heat-treating additional finely divided carbonaceous material to semi-coke the same.

3. The method of making metallurgical coke which comprises passing a stream of heating gas at a temperature between about 1,000° C. and about 1,250° C. through a travelling stream of substantially unheated carbonaceous material briquettes containing less than twenty percent of volatile substance to thereby coke said briquettes, said gas flowing around and between the briquettes in direct contact therewith regulating the rate of travel of said briquette stream and the rate of flow of said gas stream to directly heat the briquettes from about ordinary temperature at an average temperature rise between about 5° C. and 15° C. per minute to about 950° C. and reduce the mean temperature of said gas stream after its passage through said briquette stream to between about 750° C. and about 850° C., then heating with the said reduced temperature gaseous stream a mass of coal of a size substantially smaller than said briquettes to thereby remove only a part of its volatile content and to convert it into semi-coke, regulating the rate of flow of said reduced temperature gaseous stream to devolatilize the said coal at a rate by weight substantially equivalent to the rate of coking of said briquettes by the first-named heating gas stream, shaping the semi-coke thus obtained into briquettes containing less than 20% of volatile materials and supplying the said briquettes thus formed and without preliminary heating to the said stream of briquettes for coking by said first-named heating gas stream.

4. A method of making metallurgical coke according to claim 3, in which said first-named heating gas stream passes through said briquette stream transversely to the direction of travel thereof.

5. A method of making metallurgical coke according to claim 3, in which said coal is treated by the reduced temperature gaseous stream by direct contact therewith.

6. A method of making metallurgical coke according to claim 3, in which said coal is treated by the reduced temperature gaseous stream through indirect heating therefrom, said coal being conducted countercurrently to said reduced temperature gaseous stream.

7. The method according to claim 2 in which the flow of heating gas is directed alternately in one direction and in the opposite one through said stream of agglomerates.

8. A method of producing metallurgical coke which comprises heat-treating a mass of finely divided carbonaceous material to semi-coke the same, mixing the semi-cooked material with a finely-divided swelling type coal and a binder, shaping the mixture into relatively uniform size agglomerates containing less than about 20% of volatile substance, advancing said agglomerates in an initially substantially unheated state in a continuous stream flowing in one direction, bringing the agglomerates in the flowing stream into direct contact with a

highly-heated predominantly gaseous heating medium, the rate of flow of said stream of agglomerates and the temperature of the heating medium in direct contact therewith being such that they are heated at an average temperature rise of about 5° C. to 15° C. per minute to 5 increase the temperature of the agglomerates to about 950° C. to convert them into briquettes of metallurgical coke, and cooling said briquettes.

## References Cited in the file of this patent

## UNITED STATES PATENTS

|         |         |               |
|---------|---------|---------------|
| 680,780 | Knox    | Aug. 20, 1901 |
| 905,693 | Griffin | Dec. 1, 1908  |

|              |                |               |
|--------------|----------------|---------------|
| 1,276,429    | Smith          | Aug. 20, 1918 |
| 1,283,310    | Rodman         | Oct. 29, 1918 |
| 1,319,917    | Wilcox         | Oct. 28, 1919 |
| 1,490,463    | Groves et al.  | Apr. 15, 1924 |
| 5 1,597,365  | Keigley et al. | Aug. 24, 1926 |
| 1,614,028    | Hobson         | Jan. 11, 1927 |
| 1,669,023    | Runge          | May 8, 1928   |
| 1,690,933    | Hubman         | Nov. 6, 1928  |
| 1,771,048    | Koppers        | July 22, 1930 |
| 10 2,560,767 | Huff           | July 17, 1951 |
| 2,594,226    | Shea           | Apr. 22, 1952 |
| 2,619,415    | Hemminger      | Nov. 25, 1952 |
| 2,654,698    | Phinney        | Oct. 6, 1953  |